

(No Model.)

L. A. BROWN.

SEAL.

No. 392,173.

Patented Oct. 30, 1888.

Fig. 1.



Fig. 2.

Fig. 3.



Fig. 4.

Fig. 5.



Witnesses:

B. J. Re.  
W. C. Moore

Inventor:

Lewis A. Brown,  
by C. R. Moody,  
Atty.

# UNITED STATES PATENT OFFICE.

LEWIS A. BROWN, OF ST. LOUIS, MISSOURI.

## SEAL.

SPECIFICATION forming part of Letters Patent No. 392,173, dated October 30, 1888.

Application filed July 19, 1888. Serial No. 280,359. (No model.)

*To all whom it may concern:*

Be it known that I, LEWIS A. BROWN, of St. Louis, Missouri, have made a new and useful Improvement in Seals, of which the following

5 is a full, clear, and exact description.

The improvement relates to seals having or in part being composed of a label. In many forms of seals—in certain forms of car-seals, for instance—the seal is made to consist of a 10 frangible plate and a label in combination, the frangible plate being employed to guard the fastening of the lock containing the seal in such manner as to necessitate the breaking of the plate in order to reach the fastening, and the 15 label being applied to the frangible plate for the purpose of accomplishing its destruction whenever the frangible plate is broken, for should the frangible plate be broken and removed without at the same time destroying 20 the label it becomes possible to reapply the label to another frangible plate and then to substitute this second plate in the place of the original plate; but hitherto it has been found impracticable to readily so apply the label to 25 the frangible plate but that it can be removed intact therefrom. The usual form of the frangible plate is a piece of glass, and however closely a label may be gummed thereto it is not a difficult matter to separate it from the frangible 30 plate in a condition to be used again.

To obviate this difficulty and to provide an improved seal is the aim of the present improvement, which consists in a plate and a label substantially as before, but connected by 35 molding the plate onto the label—that is to say, the plate is composed of a material capable of being melted and then cast in a mold containing the label, and so as to cause the label to be fixed to a surface of the molded material. The 40 material should be, when cast, of a suitable shape and strength for the purpose in question. It should be of such a nature as not to destroy or materially impair the integrity of the label by reason of its being cast upon it. 45 It should be practically insoluble in water. It should be comparatively inexpensive, and it should have such a nature relatively to that of the material of the label as to prevent the label from being removed from it by an application 50 of moisture or by the insertion of any separa-

ting tool between the label and the plate without at the same time mutilating the label, so that the interference therewith is at once made manifest.

The improvement is best carried out in the following manner: I form a compound of sulphur, cement, and sand, taking of sulphur, by weight, nineteen parts; of cement—such as Portland—forty-nine parts; of sand, fine, thirty-two parts; heat the ingredients to a temperature of about 350° Fahrenheit, thoroughly mix them, and, at or about the temperature named, pour the compound into the mold, having first placed the label, the printed side downward, in the bottom of the mold. The label should be of a porous character, such as used in the average newspaper, and free from gum or any substance calculated to prevent the sulphur of the compound from penetrating the paper, for it is the sulphur which bonds the label so that it cannot be peeled from the plate, and if it were not desired to have a tougher stronger seal, as well as a cheaper one, the plate might be composed of sulphur only; but the cement operates to toughen and strengthen the plate and the sand to harden it and to increase its body.

The proportions named of the ingredients I consider the best to use; but it is obvious that they can be considerably varied and yet enable a valuable result to be obtained.

The plate can of course be made of various shapes. The label, while usually made of paper, it being adapted to adhere to the plate, capable of being printed and written upon, and economical in cost, can be made of any equivalent material.

In the annexed drawings, making part of this specification, Figures 1 and 2 are respectively a face and an edge view of the label; Figs. 3 and 4, respectively, a face and a section of the seal; and Fig. 5, a back view of the seal.

The label A may have any suitable inscription or marks, *a*, upon its face. The label may be coextensive with the face of the plate B; but, as shown in Figs. 3, 4, it is better to have the label somewhat smaller and countersunk in the plate. In or upon its rear face the plate B may have any mark or character, *b*, to distin-

guish its ownership or origin. The seal, especially the label portion, may be varnished to better protect it.

I claim—

5 1. A seal consisting of a plate and a label, the plate being cast onto the label, substantially as described.

2. A seal consisting of a plate and a label, the plate being composed of sulphur, cement, 10 and sand, the label being of paper, and the

plate being cast onto the label, substantially as described.

3. A seal consisting of a plate and a label, the plate containing sulphur and being cast onto the label, substantially as described.

Witness my hand.

LEWIS A. BROWN.

Witnesses:

C. D. MOODY,  
JAS. W. ALLEN.